# EUROPEAN PATENT SPECIFICATION

(11) **EP 1 495 085 B1**
(45) Date of publication and mention of the grant of the patent: **15.10.2008**
(21) Application number: 02728642.6
(22) Date of filing: 01.04.2002
(51) Int. Cl.: C09K 3/00, B05D 7/16, B32B 27/40, B05D 7/00

(54) **METALLIC FINISH**
METALLÜBERZUG
PRODUIT DE FINITION DE METAL

(43) Date of publication of application: 12.01.2005
(73) Proprietor: Lacks Enterprises, Inc., Grand Rapids, Michigan 49546 (US)
(72) Inventor: XU, Qihua (nmi), Grand Rapids, MI 49546 (US)
(74) Representative: Miller, James Lionel Woolverton
(86) International application number: PCT/US2002/010090
(87) International publication number: WO 2003/093386

(56) References cited:
- EP-A- 1 134 251
- US-A- 3 886 226
- US-A- 4 481 160
- US-A- 4 542 070
- US-A- 5 109 057
- US-A- 5 578 347
- US-B1- 6 413 588
- DATABASE WPI Section Ch, Week 199329 Derwent Publications Ltd., London, GB; Class M11, AN 1993-232842 XP002324974 & JP 05 156499 A (AISIN SEIKI KK) 22 June 1993 (1993-06-22)

## Description

### FIELD OF THE INVENTION

This invention relates to a process for depositing a polymer film on a chrome surface, and more particularly to a process for applying a durable urethane film to a chrome surface.

### BACKGROUND OF THE INVENTION

Traditional chrome plating creates a smooth, bright chrome finish. It has long been desired to have other finishes, such as black chrome, gold-tinted chrome, and other tinted or colored metallic finishes for decorative purposes. More specifically, there is a desire for clear polymeric decorative coatings that allow the brightness and luster of chrome plating to be seen, while modifying the appearance by imparting a color or tint to the chrome plating.

Several methods have been used in an attempt to achieve colored metallic finishes. One method involves electroplating, wherein black chrome and bronze finishes can be created. A problem with the electroplating methods is that it is very difficult to consistently obtain a desired colored metallic finish. Another disadvantage with the electroplating techniques is that they are generally limited to black and bronze colors or combinations thereof.

Another method that has been used for obtaining colored metallic finishes involves physical vapor deposition (PVD). This method offers a wider variety of colors than the electroplating method. However, physical vapor deposition is very expensive, and therefore, its use for achieving a desired colored finish is extremely limited. Another problem with physical vapor deposition is that it is difficult to control the gloss of the finishes.

Another method that has been attempted for obtaining colored metallic finishes involves applying a transparent organic polymer coating containing a dye, pigment or other colorant on a chrome-plated substrate. This method is convenient, and offers a very wide variety of color finishes. However, the use of organic coatings on chrome-plated substrates has been extremely limited due to poor adhesion between the organic coating and the chrome surface, especially after prolonged exposure to extreme temperature and/or humidity. Even organic polymer coating compositions which initially exhibit good adhesion have not exhibited adequate adhesive durability for most product applications. As a result, this technique has not been applied to automotive, electronic, or other durable consumer goods.

A process for adhering a relatively thick layer, e. g.,5 millimeters, of polyurethane elastomer to a metal, such as steel, iron or aluminum, is disclosed in U. S. Patent No. 4,542, 070. The process involves coating the surface of the metal with a primer composition containing a polyepoxy compound and a polyamine compound, further coating the surface with a composition containing an isocyanate compound having an isocyanate group concentration of 15-50% by weight, and casting a layer of polyurethane elastomer onto the double coated surface of the metal followed by hardening the whole system. A silane-coupling agent may be added to the primer composition to improve adhesive properties and water resistance. Disclosed examples of silane-coupling agents include gammaglycidoxypropyltrimethoxysilane and gamma- aminopropyltriethoxysilane. Color pigments may be added to the composition. Solvents that may be used for the primer composition are those which dissolve both the polyamine compound and the polyepoxy compound, with examples including toluene, xylene, ethylbenzene, methylethylketone, methylcellosolve, ethylcellosolve and acetate esters of a cellosolve compound. The polyurethane elastomer is used to improve the durability of steel, iron and aluminum surfaces of metal articles.

### SUMMARY OF THE INVENTION

In the present invention, a clear polyurethane film is adhered to a chrome surface using a primer containing an aromatic amine functional silane-coupling agent. The polymer film may contain a coloring or tinting agent that modifies the perceived color of the underlying chrome surface.

The invention offers a process of creating unique surface finishes on chrome- plated substrates. More specifically, the process provides an economical way of creating surface finishes similar to black chrome, PVD finishes, and other colored metallic finishes, such as blue, red, green, yellow, etc. The colors and the gloss level can be varied as desired. The process employs an adhesion enhancer that can be applied as a primer. The adhesion performance between the chrome surface and the film is improved so that both the film and the adhesion between the film and the chrome plating are durable enough for practical applications such as in the automotive industry and in electronic devices such as cellular phones.

These and other features, advantages and objects of the present invention will be further understood and appreciated by those skilled in the art by reference to the following specification and claims.

### DESCRIPTION OF THE PREFERRED EMBODIMENTS

In accordance with a preferred embodiment of the invention, a clear, hard polyurethane polymer film is deposited on a chrome plating by first applying an aqueous primer composition to the chrome plating, and applying a two part urethane composition over the primer composition. The primer composition is comprised, and more preferably consists essentially of, water, methanol, and an aromatic amine functional silane-coupling agent. The primer composition may be applied to a chrome surface by spraying, dipping or wiping techniques. Preferably, the chrome surface is cleaned prior to application of the primer composition. The applied primer composition is allowed to dry. After the primer composition has dried, a liquid urethane composition is applied over the dried primer composition, and is allowed to cure. The urethane composition can be applied by any of various techniques, including spraying, dipping or wiping techniques, with spraying being preferred. A suitable thermal cure can be achieved in about 60 minutes at180°F (about 82°C).

The polyurethane films made according to this invention generally have a thickness of from about 5-200 microns, more typically from 10-100 microns, and preferably from 20-50 microns.

Although a desirable aesthetic finish can be achieved without pigments or dyes, the two-part urethane composition preferably includes a dye, pigment or other colorant or a mixture of colorants to create a desired tinted film.

The urethane composition may be either a one-component urethane system, or preferably a two-component urethane system. A two-component urethane system is a urethane system in which the isocyanate and polyol components are kept separate from one another until just prior to use at which time those components are mixed together and applied to a surface. Upon mixing the two components, a full urethane polymerization reaction occurs. Generally, any of a variety of two-component polyurethane systems that are suitable for forming continuous films may be used in this invention. However, preferred polyurethane systems include those comprising, as the polyol component, alpha, omega-polymethacrylate polyols. Suitable alpha,omega-polymethacrylate polyols are commercially available, or can be obtained by reacting terminally hydroxy-functional polymethacrylates, obtained by free-radical polymerization in the presence of a hydroxy-functional molecular weigh regulator, with polyols, with the addition of non-basic transesterification catalysts, in a molar ratio of polymethacrylate to polyol of from 1:1 to 1:10. Examples of monomers that may be used for forming the polymethacrylate sequence of the terminally hydroxy-functional polymethacrylate polyols include diols such as methylmethacrylate, ethylmethacrylate, propylmethacrylate, n-butylmethacrylate, isobutylmethacrylate, tert-butylmethacrylate, n-pentylmethacrylate, amylmethacrylate, n-hexylmethacrylate, n-octylmethacrylate, 2-ethylhexylmethacrylate, n-decylmethacrylate, cyclopentylmethacrylate, cyclohexylmethacrylate, 4-tert-butylcyclohexylmethacrylate, cyclooctylmethacrylate, phenylmethacrylate, isobornylmethacrylate or other acrylates or methacrylates. Examples of suitable diols for the transesterification reaction include ethylene glycol, propane-1,2-diol, propane-1,3-diol, butane-1,2-diol, butane-1,3-diol, butane-1,4-diol, neopentylglycol, hexane-1,6-diol, octane-1,8-diol, decane-1,10-diol, doceane-1,12-diol, cyclopentane-1,2-diol, cyclohexane-1,2-diol, cyclohexane-1,4-diol, diethylene glycol, triethylene glycol, polyethylene glycol, polypropylene glycol, polybutylene glycol, polyoxyethylene-polyoxypropylene-diols, 2,3-butene-1,4-diol, 1,2-dihydroxymethylbenzene, and 1,4-dihydroxymethylbenzene. However, polyols having three or more hydroxyl functional groups may be employed.

The polyol components of the two-component urethane system may have a number-average molecular weight of from about 1,000 to about 30,000 Daltons, a hydroxyl number of between 20 and 200 mg of KOH/g, and an acid number of between 5 and 150 mg of KOH/g.

In addition to the alpha,omega-polymethacrylate polyols, other polyols may be employed. For example, to increase the hardness of the cured polyurethane film, aliphatic,
cycloaliphatic, arylaliphatic and/or aromatic diols and/or polyols, having a molecular weight of from about 60 to about 4,000 Daltons, may be employed. In order to increase flexibility of the cured urethane film, saturated and/or unsaturated polyester diols and/or polyether polyols having a number-average molecular weight of from about 400 to about 5,000 Daltons may be employed. Polyester diols may be prepared by esterifying organic dicarboxylic acids or their anhydrides with organic diols, or from a hydroxy carboxylic acid or from a lactone. Branched polyester polyols may be prepared by employing polyols or polycarboxylic acids having a higher functionality.

Other suitable polyurethane compositions may comprise, as the polyol component, various polyether polyols generally derived from cyclic ethers, and various polyester polyols, such as those obtained from residues of terephthalic acid production or by transesterification of dimethyl terephthalate or poly(ethylene terephthalate) with glycols.

Examples of suitable polyisocyanate compounds that may be used in the two-component urethane systems include monomeric organic polyisocyanates having a molecular weight of from about 140 to 300 Daltons, lacquer polyisocyanates having a molecular weight of from about 300 to 1,000 Daltons, and isocyanate-functionalized prepolymers containing urethane groups and having a molecular weight above 1,000 Daltons, as well as mixtures thereof.

Examples of monomeric polyisocyanates include 1,4-diisocyanato-butane, 1,6-diisocyanatohexane, 1,5-diisocyanato-2,2-dimethyl-pentane, 2,2,4-trimethyl-1,6-diisocyanatohexane, 2,4,4-trimethyl-1,6-diisocyanatohexane, 1-isocyanato-3,3,5-trimethyl-5-isocyanatomethylcyclohexane, 1-isocyanato-1-methyl-4(3)-isocyanatomethylcyclohexane, bis-(4-isocyanatocyclohexyl)methane, 1,10-diisocyanatodecane, 1,12-diisocyanatododecane, cyclohexane-1,3-diisocyanate, cyclohexane-1,4-diisocyanate, xylylenediisocyanate isomers, 2,4-diisocyanatotoluene and mixtures thereof with 2,6-diisocyanatotoluene, 2,2'-diisocyanatodiphenylmethane, 2,4'-diisocyanatodiphenylmethane, 4,4'-diisocyanatodiphenylmethane, and mixtures of the preceding polyisocyanates. Lacquer polyisocyanates are obtained by oligomerizing monomeric diisocyanates to form carbodiimide, uretdione (dimers), isocyanurate (trimers), biuret, urea, urethane, allophanate and/or oxadiazine groups. Several of these groups may be formed simultaneously or successively during oligomerization.

Examples of isocyanate functionalized prepolymers containing urethane groups having a molecular weight of about 1,000 or above may be prepared by reacting monomeric diisocyanates and/or lacquer polyioscyanates with an organic polyhydroxyl compound having a molecular weight of about 300 or greater. The polyhydroxyl compounds typically used to prepare isocyanate functionalized prepolymer are those having a number average molecular weight that is preferably greater than 500 Daltons, and more preferably from about 500 Daltons to about 4,000 Daltons. These polyhydroxyl compounds typically have from 2 to 6, and more typically from 2 to 3 hydroxyl groups from molecule, and are generally selected from ether, ester, thioether, carbonate and/or polyacrylate polyols.

To prepare a two-component coating composition for use in practicing this invention, one or more polyols, and one or more polyisocyanates are mixed together in amounts corresponding to an NCO : OH equivalent ratio of from about 0.5 : 1 to about 2.0 : 1, more typically from about 0.8 : 1 to about 1.5 : 1. Various ingredients conventionally employed in urethane coating compositions may be added. These ingredients include flow control agents, viscosity-controlling additives, pigments, fillers, flatting agents, UV stabilizers and anti-oxidants and catalysts for the cross-linking reaction.

Although two-component urethane systems are preferred, one-component urethane systems may also be used. One-component urethane systems are those in which a soluble or dispersible urethane prepolymer that is the reaction product of a polyol with a polyisocyanate is provided with moisture curable functionalities or airdrying functionalities that facilitate cross-linking and formation of a film after application to a chrome substrate. Examples of one-component urethane systems include air-curing urethanes systems such as those in which an oligomeric urethane prepolymer is cross-linked by oxidation of unsaturated carbon-carbon double bonds in a long chain aliphatic group. Other one-component urethane systems include moisture curable urethane systems that include silanol terminated urethane prepolymers that are cross-linked by hydrolysis and silane condensation reactions upon contact with moisture.

Generally, two-component urethane compositions are preferred because they usually exhibit better scratch resistance, and chemical resistance than one-component systems. However, the principels of this invention may be applied to other applications using a one-component urethane system when scratch-resistance and chemical resistance are not as important as it is with most automotive and electronic applications (e. g., cellular telephone housings).

The polyurethane films made according to this invention are preferably relatively hard and non- elastomeric, and exhibit a pencil hardness of from about 3H to about 6H.

Depending on the selection of polyisocyanates, polyols, and additives, the coating composition may be solventless, aqueous-based, or organic solvent-based.

The description is intended to provide examples of suitable polyols and polyisocyanates that may be employed in the practice of this invention. However, the invention is not limited to any particular two-component polyurethane systems. Two- component urethane systems containing acrylic polyols such as polymeric/oligomeric materials comprised of acrylates, methacrylates, acrylonitrile, methacrylonitrile, or combinations of these monomers etc. are suitable and/or preferred. However, other polyurethane compositions such as polyether based urethane systems are also believed to be suitable for various automotive, appliance and consumer electronics applications.

Generally any of a variety of commercially available two-component urethane compositions may be employed in accordance with this invention to provide an aesthetic or functional film that is strongly adhered to a chrome surface.

The silane adhesion enhancer may be employed in a primer composition in an amount of from about 0. 05 to about 5 %, and more preferably from about 0.5 to about 2 %, by weight of the primer composition, with an amount of 1 % being most preferred. Preferably, the primer composition is an aqueous solution that is free, or at least substantially free, of environmentally undesirable volatile organic compounds. Preferably, the aqueous primer composition is comprised of, and more preferably consists essentially of, water, methanol, and one or more aromatic amine functional silane adhesion enhancers. The aqueous primer composition may contain from about 50 % to about 95 % water, and from about 5 to 50 % methanol.

Preliminary testing has strongly suggested that aromatic amine functional silane-coupling agents, such as N-phenyl-gamma-aminopropyltrimethoxysilane are particularly useful as adhesion enhancers for achieving strong, durable adhesion between a chrome plate and a cured polyurethane film. A variety of suitable aromatic amine functional silane-coupling agents are well known and commercially available.

A particular use of this invention involves application of a tinted or colored decorative polymer film to a chrome plate to impart a desired hue or color to the chrome plate while also allowing the brightness and luster of the chrome plate to be seen through the film. Therefore, in accordance with this aspect of the invention, any of various dyes, pigments, or other colorants, or mixtures of colorants may be added in an amount effective to impart a desired color, tint or hue to a chrome plate. Suitable colorants and amounts thereof are well known and/or can be easily determined by routine experimentation. The tinted urethane compositions to be used according to this invention, when applied to a chrome plate, create a unique surface finish that is different from conventional paint or traditional chrome plated finishes. The tinted finishes can be generally any color in the spectrum, e. g., gray, gold, red, blue, etc.

Preliminary testing has shown that urethane coatings applied to a chrome substrate in accordance with this invention demonstrate outstanding adhesion even after an extended period of time under a humid environment.

The following examples are illustrative of certain aspects of the invention.

Adhesion tests were conducted on coated samples using the compositions and processes of this invention (Example 3) and compared with the adhesion results of a conventional urethane coating composition (Example 4) and with a prior art composition (Example 2). Adhesion testing was conducted by keeping coated samples at ambient temperature for at least 4 hours, then immersing the samples in water at 38°C for 10 days. Thereafter a grid pattern was cut into each sample. The lines in the grid pattern were 2 mm apart from each other. A pressure sensitive adhesive tape was used to evaluate adhesion. The average percentage of coating that remained after the tape was pressed onto the grid and peeled away was used as an indication of adhesive strength or quality. Comparative Example 1 describes preparation of a primer solution according to the prior art.

### Comparative Example 1-Preparation of Primer Solution 1

In a clean beaker, 50 ml methanol, 7 ml of A-187 silane (gammaglycidoxypropyltrimethoxysilane), available from OSI Specialties, and 3 ml ofA 1170 silane[bis- (gamma-trimethoxysilylpropyl) amine], available from OSI Specialties, was added. The solution was stirred for 5 minutes at room temperature. The solution was allowed to age overnight at room temperature. In a separate beaker, 200ml of isopropyl alcohol and 25 ml de-ionized water were combined. Then 6 ml of solution 1 was added under stirring. The primer solution was allowed to age for 4 hours at room temperature before use.

### Comparative Example 2

On 10 cm x 10 cm (4"x 4") chrome-plated plaques, the primer solution 1 was applied by dipping and dried for 5 minutes at room temperature. A two-part urethane clear coating (SL201 from Red Spot Paint & Vanish) was mixed based on the suggested ratio and applied by spray and cured for 1 hour at 82°C (180 F). The adhesion tested by adhesion tape was improved after a temperature and humidity cycle as compared with a control (Example 4). More specifically, the average percentage of coating that remained after the tape was removed was about 90 %, as compared with about 50 % for the conventional urethane coating.

### Example 3

A two-part urethane clear coating (SL201 from Red Spot Paint & Vanish) was mixed based on the suggested ratio. Silane Y-6996 (N-phenyl-gamma-aminopropyltrimethoxysilane), available from OSI Specialities, was added at 0.5% to the total mixed paint by volume. The coating was applied by spraying on the chrome-plated plaques and cured for 1 hour at 82°C (180 F). The adhesion tested by adhesion tape was improved after a temperature and humidity cycle as compared with a control (Example 4). More specifically, the average percentage of coating that remained after the tape was removed was about 100%, as compared with about50 % for the conventional urethane coating.

### Example 4 (Control)

The two-part urethane clear coating used in Example 3 was applied by spray on the chrome**-**plated plaques and cured for 1 hour at 82°C (180 F). The adhesion tested by adhesion tape was poor after a temperature and humidity cycle. More specifically, the average percentage of coating that remained after the tape was removed was about 50%.

The above description is considered that of the preferred embodiments only. Modifications of the invention will occur to those skilled in the art and to those who make or use the invention.

## Claims

1. A process for forming a polyurethane film on a chrome plate, comprising:
applying an aqueous primer composition to the chrome plate, the primer composition containing at least one silane adhesion promoter selected from aromatic amine functional silane-coupling agents;
drying the applied primer composition;
applying a urethane composition over the chrome plate on which the aqueous primer was applied and dried; and
curing the urethane composition to form a polyurethane film.

2. The process of claim 1, wherein the aromatic amine functional silane-coupling agent is N-phenyl-gamma-aminopropyltrimethoxysilane.

3. The process of claim 1 or claim 2, wherein the silane adhesion promoter is present in the aqueous primer composition in an amount of from about 0.05 % to about 5 % by weight.

4. The process of any preceding claim, wherein the silane adhesion promoter is present in the aqueous primer composition in an amount of from about 0.5% to about 2% by weight.

5. The process of any preceding claim, wherein the silane adhesion promoter is present in the aqueous primer composition in an amount of about 1 % by weight.

6. The process of any preceding claim, wherein the urethane composition includes a polymethacrylate polyol.

7. The process of any preceding claim, wherein the urethane composition further comprises a colorant in an amount effective to impart a desired color, tint or hue to the chrome plate.

8. The process of any preceding claim, wherein the polyurethane film has a thickness of from 5-200 microns.

9. The process of any preceding claim, wherein the polyurethane film has a pencil hardness of from about 3H to 6H.

10. An article comprising:
a chrome plate;
a polyurethane film adhered to the chrome plate; and
the residue of a silane adhesion promoter enhancing adhesion between the polyurethane film and the chrome plate, wherein the silane adhesion promoter included at least one silane adhesion promoter selected from aromatic amine functional silane-coupling agents.

11. The article of claim 10, wherein the aromatic amine functional silane-coupling agent was N-phenyl-gamma-aminopropyltrimethoxysilane.

12. The article of any one of claims 10 to 11, wherein the polyurethane film further comprises a colorant in an amount effective to impart a desired color, tint or hue to the chrome plate.

13. The article of any one of claims 10 to 12, wherein the polyurethane film has a thickness of from 5-200 microns.

14. The article of any one of claims 10 to 13, wherein the polyurethane film has a pencil hardness of from about 3H to 6H.

## Patentansprüche

1. Verfahren zum Bilden eines Polyurethanfilms auf einer Chromplatte, welches umfasst:
Auftragen einer wässerigen Grundierungszusammensetzung auf die Chromplatte, wobei die Grundierungszusammensetzung mindestens einen Silan-Adhäsionspromotor enthält, ausgewählt aus aromatischen Amin-funktionellen Silan-Haftvermittlern;
Trocknen der aufgetragenen Grundierungszusammensetzung;
Auftragen einer Urethanzusammensetzung über die Chromplatte, auf welche die wässerige Grundierung aufgetragen und getrocknet wurde; und
Härten der Urethanzusammensetzung, um einen Polyurethanfilm zu bilden.

2. Verfahren nach Anspruch 1, worin der aromatische Aminfunktionelle Silan-Haftvermittler N-Phenyl-gammaaminopropyltrimethoxysilan ist.

3. Verfahren nach Anspruch 1 oder Anspruch 2, worin der Silan-Adhäsionspromotor in der wässerigen Grundierungszusammensetzung in einer Menge von etwa 0,05 Gew.-% bis etwa 5 Gew.-% vorhanden ist.

4. Verfahren nach einem vorhergehenden Anspruch, worin der Silan-Adhäsionspromotor in der wässerigen Grundierungszusammensetzung in einer Menge von etwa 0,5 Gew.-% bis etwa 2 Gew.-% vorhanden ist.

5. Verfahren nach einem vorhergehenden Anspruch, worin der Silan-Adhäsionspromotor in der wässerigen Grundierungszusammensetzung in einer Menge von etwa 1 Gew.-% vorhanden ist.

6. Verfahren nach einem vorhergehenden Anspruch, worin die Urethanzusammensetzung ein Polymethacrylatpolyol einschließt.

7. Verfahren nach einem vorhergehenden Anspruch, worin die Urethanzusammensetzung ferner einen Farbstoff in einer Menge umfasst, welche wirksam ist, der Chromplatte eine gewünschte Farbe, Färbung oder Farbschattierung zu verleihen.

8. Verfahren nach einem vorhergehenden Anspruch, worin der Polyurethanfilm eine Dicke von 5-200 Mikron hat.

9. Verfahren nach einem vorhergehenden Anspruch, worin der Polyurethanfilm eine Bleistiftritzhärte von etwa 3H bis 6H hat.

10. Artikel, umfassend:
eine Chromplatte;
einen an der Chromplatte angehafteten Polyurethanfilm; und
den Rückstand eines Silan-Adhäsionspromotors, welcher Adhäsion zwischen dem Polyurethanfilm und der Chromplatte erhöht, worin der Silan-Adhäsionspromotor mindestens einen Silan-Adhäsionspromotor, ausgewählt aus aromatischen Amin-funktionellen Silan-Haftvermittlern einschloss.

11. Artikel nach Anspruch 10, worin der aromatische Aminfunktionelle Silan-Haftvermittler N-Phenyl-gammaaminopropyltrimethoxysilan war.

12. Artikel nach einem von Ansprüchen 10 bis 11, worin der Polyurethanfilm ferner einen Farbstoff in einer Menge umfasst, welche wirksam ist, der Chromplatte eine gewünschte Farbe, Färbung oder Farbschattierung zu verleihen.

13. Artikel nach einem von Ansprüchen 10 bis 12, worin der Polyurethanfilm eine Dicke von 5-200 Mikron hat.

14. Artikel nach einem von Ansprüchen 10 bis 13, worin der Polyurethanfilm eine Bleistiftritzhärte von etwa 3H bis 6H hat.

## Revendications

1. Procédé de formation d'un film de polyuréthane sur un dépôt de chrome, comprenant les étapes consistant à :
appliquer une composition de couche de fond aqueuse sur le dépôt de chrome, la composition de couche de fond contenant au moins un promoteur d'adhérence à base de silane choisi parmi des agents d'accrochage à base de silane aminofonctionnel aromatique ;
sécher la composition de couche de fond appliquée ;
appliquer une composition à base d'uréthane sur le dépôt de chrome sur lequel la couche de fond aqueuse a été appliquée et séchée ; et
faire durcir la composition à base d'uréthane pour former un film de polyuréthane.

2. Procédé selon la revendication 1, dans lequel l'agent d'accrochage à base de silane aminofonctionnel aromatique est du N-phényle-gamma-aminopropyltriméthoxysilane.

3. Procédé selon la revendication 1 ou 2, dans lequel le promoteur d'adhérence à base de silane est présent dans la composition de couche de fond aqueuse dans une proportion allant d'environ 0,05% à environ 5% en poids.

4. Procédé selon l'une quelconque des revendications précédentes, dans lequel le promoteur d'adhérence à base de silane est présent dans la composition de couche de fond aqueuse dans une proportion allant d'environ 0,5% à environ 2% en poids.

5. Procédé selon l'une quelconque des revendications précédentes, dans lequel le promoteur d'adhérence à base de silane est présent dans la composition de couche de fond aqueuse dans une proportion d'environ 1% en poids.

6. Procédé selon l'une quelconque des revendications précédentes, dans lequel la composition d'uréthane comprend un polyol de polyméthacrylate.

7. Procédé selon l'une quelconque des revendications précédentes, dans lequel la composition d'uréthane comprend en outre un colorant dans une proportion suffisant à donner une couleur, teinte ou nuance voulue au dépôt de chrome.

8. Procédé selon l'une quelconque des revendications précédentes, dans lequel le film de polyuréthane a une épaisseur allant de 5 à 200 microns.

9. Procédé selon l'une quelconque des revendications précédentes, dans lequel le film de polyuréthane a une dureté au crayon d'environ 3H à 6H.

10. Article, comprenant :
un dépôt de chrome ;
un film de polyuréthane adhéré sur le dépôt de chrome ; et
le résidu d'un promoteur d'adhérence à base de silane améliorant l'adhérence entre le film de polyuréthane et le dépôt de chrome, dans lequel le promoteur d'adhérence à base de silane comprend au moins un promoteur d'adhérence à base de silane choisi parmi des agents d'accrochage à base de silane aminofonctionnel aromatique.

11. Article selon la revendication 10, dans lequel l'agent d'accrochage à base de silane aminofonctionnel aromatique est du N-phényle-gamma-aminopropyltriméthoxysilane.

12. Article selon l'une quelconque des revendications 10 à 11, dans lequel le film de polyuréthane comprend en outre un colorant dans une proportion suffisant à donner une couleur, teinte ou nuance voulue au dépôt de chrome.

13. Article selon l'une quelconque des revendications 10 à 12, dans lequel le film de polyuréthane a une épaisseur allant de 5 à 200 microns.

14. Article selon l'une quelconque des revendications 10 à 13, dans lequel le film de polyuréthane a une dureté au crayon allant d'environ 3H à 6H.
